

July 3, 1962

J. W. LYLE

3,041,672

## MAKING SPHEROIDAL POWDER

Filed Sept. 22, 1958



Fig. 5

INVENTOR  
JAMES W. LYLE  
BY  
Barrett P. King  
ATTORNEY

# United States Patent Office

3,041,672

Patented July 3, 1962

1

3,041,672

## MAKING SPHEROIDAL POWDER

James W. Lyle, Indianapolis, Ind., assignor to Union Carbide Corporation, a corporation of New York  
Filed Sept. 22, 1958, Ser. No. 762,296  
6 Claims. (Cl. 18—47.3)

This invention relates to powder making, and more particularly to the production of finely divided, spheroidal shaped powder particles.

There exists a commercial need for fine powders which are reasonably uniform in size and spheroidal in shape. Such powders can be more readily dispensed and handled. Processes employing such powders thus have a more uniform raw material with which to deal. Spheroidal shaped particles are usually preferred in contrast to irregular shaped particles obtained by mechanical grinding methods.

A novel process has been developed, according to this invention, for producing fine particles of spheroidal shape. This process comprises the steps of striking an arc between a stick electrode and a nozzle electrode, said arc being wall-stabilized at least along a portion of its length, introducing a consumable wire or rod into the collimated plasma effluent of such arc, passing a gas stream along and coextensive with such collimated plasma to shear off molten material from the molten surface of the consumable wire whereby small droplets are formed and removed from the arc zone, and then solidifying and collecting the so-produced finely-divided particles.

A wall-stabilized and constricted arc of the type used in this invention is described more fully in U.S. Patent No. 2,806,124 and copending application S.N. 539,794, now Patent No. 2,858,411, dated October 28, 1958.

The preferred operating condition for smallest particle size of product involves introducing the consumable wire or rod within the nozzle electrode passage at the point of maximum arc construction and maximum momentum of the arc plasma and coextensive gas stream. The gas stream employed should preferably be chemically inert to the molten particles so as to prevent reaction between the gas and particles in addition to shielding the hot particles from atmospheric oxidation. In addition, for maximum melt-off rates of the consumable wire and highest production rates for fine powder, the consumable wire is preferably an electrode carrying the bulk of the arc current.

This process is especially useful for producing finely divided, spheroidal-shaped metal particles. However, it may also be employed with metal compounds, such as the refractory metal oxides, silicides, borides, nitrides and carbides, which are difficult if not impossible to produce in fine spheroidal form by prior art techniques.

These fine particles are relatively uniform in shape and size. Their actual size appears to be dependent upon arc power and gas momentum. The spheroidal shape renders these products more free-flowing than prior art irregular shaped particles obtained by mechanical grinding methods. They are also useful for producing sintered porous bodies having relatively uniform pore size.

This process has the additional advantage of producing fine powders of material which has such a high degree of ductility that it cannot be mechanically ground. Also, it can produce powders of refractory materials which cannot be readily melted and treated in conventional shot-tower processes.

In the drawings:

FIG. 1 is a fragmentary view in vertical cross-section of apparatus for making powder according to the invention; and

FIGS. 2-5 are similar views of other modifications.

2

Referring to FIG. 1, an arc is struck between stick electrode 10 and nozzle electrode 11. Electrical power is supplied from source 12 through leads 13 and 14. A gas stream passes down along electrode 10 and forces the arc 15 down into the constricted portion 16 of the nozzle passage 17 where the arc becomes wall-stabilized. The nozzle electrode 11 is cooled below its melting point by passing cooling fluid, such as water, from inlet 28 through passage 29 to outlet 30.

- 10 A consumable wire 18 is preferably introduced at or near the point of maximum nozzle constriction and maximum arc plasma momentum in order to obtain fine particle size product. This process is not limited, however, to wire introduction at this point. The wire may be introduced at other points in the nozzle or at the nozzle outlet as shown in the position of wire 19 of FIG. 2. When the wire 18 is introduced as shown in FIG. 1, the nozzle passage extending beyond the point of wire entry tends to improve results by focusing and controlling the position of the molten droplet stream. It also directs the gas stream and maintains improved shielding of the metal particles from atmospheric contamination. A divergent discharge passage 20 is conveniently employed primarily to reduce the possibility of nozzle plugging caused by 15 deposits of molten metal particles. It also prevents the formation of an undesirable shock front at the outlet which can occur with straight nozzles. A divergent nozzle passage is desirable in that it spreads the nozzle electrode area and reduces current density. This helps 20 reduce nozzle erosion at high current levels. It is preferred for the above reasons that the nozzle outlet have an increased cross-sectional area as compared to the area of the nozzle at the point of wire entry. Nozzle shapes other than that shown might also be used. The 25 molten particles 21 entrained in the torch gas stream pass out of the apparatus and are solidified and collected in a collector 22. This collector may, for example, contain a body of water into which the molten particles are directed for solidification.
- 30 In the apparatus modification shown in FIG. 1 the wire 18 can be in electrical contact with nozzle electrode 11 and thus become an electrode. When the wire extends into the nozzle passage the arc current can terminate at the wire instead of the nozzle. This increases wire 35 melt-off and increases production rates of fine particles.
- 35 Another modification of apparatus suitable for carrying out the present novel process is shown in FIG. 3. In this form the consumable wire 18 is electrically insulated from nozzle electrode 11 by insulator 23. The 40 wire 18 can then be out of the electrical circuit, or in the preferred form can be almost electrically independent of the nozzle. The main electrical connections in the preferred form of this modification are from the power supply 12 through lead 13 to the stick electrode 10 and lead 24 to the consumable wire 18. The nozzle electrode 11 is connected to the power supply through resistance 45 25 which tends to maintain the nozzle at a lower potential than that of the consumable wire. This apparatus can be operated at higher wire feed rates than that of FIG. 1 because higher power levels can be maintained to the wire without damage to the nozzle. This becomes 50 important when wire feed rates as high as 100 lbs./hr. are desired. A pilot arc is maintained between the stick electrode and the nozzle electrode in order to effect start-up of the process and also to maintain an arc if wire feed ceases for any reason. The electrical contact from lead 55 24 to wire 18 is conveniently positioned externally to the torch in order to increase resistance heating along the wire and increase melt-off rates.
- 60 In order to fully protect the molten particles from atmospheric contamination prior to their solidification,

additional shielding gas can be introduced through shielding means 26 shown in FIG. 3. An alternative method is to completely inclose the path of the molten particles from the torch to the collector 22 by shielding means 27 shown in FIGS. 4 and 5.

The following examples are illustrative of the present process in operation.

### EXAMPLE I

#### Production of Finely-Divided Steel Particles

An apparatus of the type shown in FIG. 1 was used consisting of a  $\frac{1}{16}$ -inch dia. throttled tungsten stick cathode and a water cooled nozzle anode having a throat section  $\frac{1}{16}$ -inch dia. and  $\frac{3}{4}$ -inch long. The nozzle passage beyond the throat was  $\frac{5}{8}$ -inch long having a  $30^\circ$  divergent angle. The stick cathode was set back  $\frac{1}{8}$ -inch from the throat section. An arc of 150 amperes and 85 volts was maintained between the stick cathode and nozzle anode while a gas mixture of 200 c.f.h. argon and 13.5 c.f.h. hydrogen passed along the tungsten cathode and out through the nozzle passage. A  $\frac{1}{16}$ -inch dia. steel wire (Linde No. 65 welding wire) was introduced at a rate of about 7 lbs./hr. to the nozzle passage at a point adjacent to the throat section. The wire was in electrical contact to the nozzle anode and thus became an effective anode as it projected into the nozzle passage. The molten particles from the wire were entrained in the gas stream and were collected in a container of water positioned about 1-ft. from the torch outlet. The resulting product particles were substantially all spherical in shape with an average size of about 6 microns.

### EXAMPLE II

#### Production of Finely-Divided Steel Particles

The same equipment was used as described in Example I above. An arc of 150 amperes and 68 volts was maintained between the stick cathode and nozzle anode while a gas mixture of 200 c.f.h. argon and 13.5 c.f.h. hydrogen passed along the tungsten cathode and out through the nozzle passage. A  $\frac{1}{16}$ -inch dia. steel wire was introduced at a rate of about 5.9 lbs./hr. to the nozzle passage at a point adjacent to the throat section. The wire was in electrical contact with the nozzle and thus became an effective anode as it projected into the nozzle passage. The molten particles from the wire were entrained in the gas stream and were collected in a container of water positioned about 1-ft. from the torch outlet. The resulting product particles were substantially all spherical in shape with an average size of about 185 microns.

### EXAMPLE III

#### Production of Finely-Divided Tungsten Particles

The same basic equipment described in Example I above was used. In addition a brass tube 2-in. I.D. and 4-ft. long was attached to the torch outlet. The outlet end of this tube was immersed in water. This is shown in FIG. 5. An arc of 125 amperes and 75 volts was maintained between the stick cathode and nozzle anode while a gas mixture of 200 c.f.h. argon and 13.5 c.f.h. hydrogen passed through the torch. A  $\frac{1}{16}$ -inch dia. tungsten wire was introduced at a rate of about 4.8 lbs./hr. to the nozzle passage adjacent to the throat section. The wire was in electrical contact with the nozzle and thus became an effective anode as it projected into the passage. The molten particles from the wire were entrained in the gas stream and were solidified and collected in the water located at the end of the protective tube. The product particles were substantially all spherical in shape with an average diameter of 380 microns.

### EXAMPLE IV

#### Production of Finely-Divided Sapphire Particles

Equipment described in Example I above was used. An arc of 140 amperes and 85 volts was maintained be-

tween the stick cathode and nozzle anode while a gas mixture of 200 c.f.h. argon and 13.5 c.f.h. hydrogen passed along the tungsten cathode and out through the nozzle passage. A  $\frac{1}{16}$ -inch dia. sapphire rod was introduced to the nozzle passage at a point adjacent to the throat section. The rod was non-conducting and was thus not in the electrical circuit. The molten particles from the rod were entrained in the gas stream and were collected in a container of water positioned about 1-ft. from the torch outlet. The resulting product particles were substantially all spherical in shape with an average particle size of about 6 microns.

### EXAMPLE V

#### Production of Finely-Divided Sapphire Particles

A run similar to that of Example IV was made at 30 volts and 130 amperes with 100 c.f.h. argon gas. The  $\frac{1}{16}$ -inch dia. sapphire rod formed spherical particles with an average particle size of 12 microns.

Control of the average size of the particles produced by this process can be obtained through control of arc power and gas momentum. Dependency of particle size on arc power is shown in the following table. The gas flow remained constant and the wire feed rate was adjusted to compensate for difference in melting rates caused by different arc power.

Table I  
EFFECT OF ARC POWER ON PARTICLE SIZE

|    | Voltage, Volts | Current, Amps. | Power, kw. | Average Particle Size, Microns |
|----|----------------|----------------|------------|--------------------------------|
| 35 | 68             | 200            | 13.6       | 107                            |
|    | 68             | 150            | 10.2       | 185                            |
|    | 68             | 100            | 6.0        | 393                            |

Dependency of particle size on gas momentum is shown below. The arc power remained substantially constant and the wire feed rate was adjusted as required.

Table II  
EFFECT OF GAS FLOW ON PARTICLE SIZE

|    | Gas Flow         |               | Average Particle Size, Microns |
|----|------------------|---------------|--------------------------------|
|    | Hydrogen, c.f.h. | Argon, c.f.h. |                                |
| 50 | 13.5             | 200           | 203                            |
|    | 13.5             | 300           | 182                            |

It can be seen from the above tables that as the arc power and the gas momentum through the torch, as indicated by total gas flow through the torch, are increased, the average particle size decreases.

The fine spheroidal particles produced by the present invention may be used as starting materials for miniature ball bearings or in powder metallurgy for making sintered porous bodies of relatively uniform pore size. This novel process has the additional advantage of producing fine powders of material, such as nickel-chromium alloy, which has such a high degree of ductility that it cannot be mechanically ground. Also, it can produce powders of refractory materials, such as tungsten carbide, which cannot be readily melted and treated in conventional shot-tower processes.

What is claimed is:

1. Method of producing finely-divided spheroidal-shaped particles of metals and metal compounds by striking a wall-stabilized arc between a stick electrode having an arc constricting passage and a nozzle electrode, introducing a consumable wire or rod composed of said metals and metal compounds into the collimated plasma effluent of such arc, passing a gas stream coextensive with

such collimated plasma through the nozzle passage of the nozzle electrode to shear off molten material from the tip of the consumable wire whereby small droplets are formed and removed from the arc zone, and then solidifying and collecting the so-produced finely-divided particles.

2. Method of producing finely-divided spheroidal-shaped particles of metals and metal compounds by striking a wall-stabilized arc between a stick electrode and a nozzle electrode having an arc constricting passage, introducing a consumable wire or rod composed of said metals and metal compounds into the collimated plasma effluent of such arc, passing a gas stream coextensive with such collimated plasma through the nozzle passage of the nozzle electrode to shear off molten material from the tip of the consumable wire whereby small droplets are formed and removed from the arc zone, and then solidifying and collecting the so-produced finely-divided particles, in which the preferred operating condition for smallest particle size involves introducing the consumable metal wire at the point of maximum arc constriction and maximum momentum of the arc plasma and coextensive gas stream.

3. Method as defined by claim 2, in which, for maximum melt-off rates of the consumable wire and highest production rates for fine powder, the consumable wire is preferably an electrode carrying the bulk of the arc current.

4. Process as defined by claim 2, in which such arc effluent is conically expanded and thereby is focussed downwardly in the direction of a liquid in a container

disposed thereunder for collecting such spray of individual spheroids.

5. Process as defined by claim 4, in which such wire is laterally fed into one side of such downwardly focussed effluent so that such particles are sheared therefrom by such arc effluent which comprises inert gas.

6. The method of producing very small spheroidal-shaped particles of metals and metal compounds by striking an arc between a first nonconsumable electrode and a second constricting nonconsumable nozzle electrode having an expanding conical outlet, passing a gas stream in contact with said electrodes and through said nozzle electrode to produce a collimated plasma effluent, introducing a consumable wire or rod of said metals and metal compounds into the collimated plasma at a point of maximum arc constriction and plasma momentum, whereby said wire is melted and disintegrated into small droplets and removed from the arc zone by the plasma stream, and then solidifying and collecting the resulting spheroidal powder particles.

References Cited in the file of this patent

UNITED STATES PATENTS

|           |                |                |
|-----------|----------------|----------------|
| 1,128,175 | Morf           | Feb. 9, 1915   |
| 1,133,508 | Schoop         | Mar. 30, 1915  |
| 2,189,387 | Wissler        | Feb. 6, 1940   |
| 2,269,528 | Gallup         | Jan. 13, 1942  |
| 2,768,279 | Rava           | Oct. 23, 1956  |
| 2,770,708 | Briggs         | Nov. 13, 1956  |
| 2,795,819 | Lezberg et al. | June 18, 1957  |
| 2,806,124 | Gage           | Sept. 10, 1957 |